

3,287,132

## SILVER DYE BLEACH DYESTUFFS AND THEIR USE IN COLOUR PHOTOGRAPHY

Francis George Hunt, Huddersfield, England, assignor to Ilford Limited, Ilford, England, a British company  
 No Drawing. Filed Sept. 5, 1963, Ser. No. 306,685  
 Claims priority, application Great Britain, Sept. 24, 1962,  
 36,242/62

11 Claims. (Cl. 96—53)

This invention relates to dyestuffs and to their use in colour photography and particularly in the silver-dye-bleach process of colour photography.

In this process a photographic silver halide emulsion layer, usually a gelatino silver halide emulsion layer, includes as a uniform dispersion therein, a suitable dyestuff. A latent silver image is formed in the layer and is developed to a silver image. The layer is then treated with a "bleach" bath which has the effect of oxidising the silver image and simultaneously reducing (bleaching) the dyestuff in the region of the silver image. The silver salts and any residual silver are then removed and the layer then contains only a dyestuff image which is complementary in sign to the original silver image.

Variations are possible in this process. For example, the layer may be dyed with the dyestuff after the exposure step or after the development of the silver image, or the dyestuff may be included in a plain gelatin layer coated adjacent to the emulsion layer. A large number of patents have been granted in respect of the process, the main details of which can be ascertained from British patent specifications Nos. 397,159 and 397,188.

In order to produce a record in full colour there is generally employed a multilayer material which contains three light-sensitive silver halide emulsion layers, one sensitive to blue light only and the other sensitised to green and red light respectively. To prevent these latter layers from recording blue light in addition to the light to which they are sensitised, it is usual to provide a blue-absorbing filter layer between these latter layers and the emulsion which is sensitive only to blue, a common form of assembly being:

- Support layer
- Red-sensitive emulsion layer
- Green-sensitive emulsion layer
- Blue-absorbing filter layer
- Blue-sensitive emulsion layer.

Layer (d) is not always essential since layer (e), when dyed yellow, may provide a sufficient barrier to blue light.

Polychromatic light incident on layer (e) causes the formation of latent silver images in layers (e), (c) and (b), respectively recording in those layers the blue, green and red sensations of the exposing light.

In the silver-dye-bleach process as ordinarily practised, layer (b) is dyed blue-green (cyan), layer (c) is dyed magenta and layer (e) is dyed yellow. Accordingly, when the material is exposed, developed to form silver images and subjected to the required bleaching treatment and treated to remove residual silver salts and silver, the final product carries "positive" yellow magenta and cyan images complementary to the "negative" silver images formed on development, so that when viewed it provides an accurate representation of the original subject of the exposure.

A principal difficulty associated with the process is to ensure that the dyestuff employed will not diffuse from the gelatin emulsion layer in which it is incorporated, and various proposals, such as mordanting, have been made to overcome this difficulty. In selecting dyestuffs for use, moreover, it is desirable that they should be bleached

rapidly by the bleaching baths employed and also important that their inclusion in the emulsion layer should not too seriously reduce the sensitivity of the emulsion. In addition, of course, it is desirable that the dye should approach as closely as possible to the theoretical requirement that, of red, blue and green light, it should absorb all of one while fully transmitting or reflecting both of the others.

It is an object of the present invention to provide a new class of cyan dyestuffs for use in the silver-dye-bleach process which closely approach the desiderata set forth above.

According to a first feature of the present invention there are provided cyan dyestuffs of the general Formula

15 I:



where X is halogen, hydroxyl, amino, substituted amino or hydrogen, the ring W is unsubstituted or carries one or more substituents selected from halogen, alkyl, alkoxy, sulphonic acid and alkali metal sulphonate, the number of sulphonic acid or sulphonate groups in the ring W being not greater than 1, U is hydrogen, sulphonic acid or alkali metal sulphonate, V is hydrogen or the group

20 ing



and R<sub>1</sub> and R<sub>2</sub> are hydrogen, alkyl, substituted alkyl (e.g.  $\beta$ -hydroxy ethyl), cycloalkyl, aralkyl or aryl, or R<sub>1</sub> and R<sub>2</sub> together constitute, with the nitrogen atom to which they are attached, a cyclic grouping, e.g. morpholino.

The aforesaid dyes may be prepared by the method in which the diazotised p-nitroaniline derivative (or p-aminoacetanilide derivative) is coupled to the first naphthalene component, the monoazo compound is reduced (or hydrolysed), re-diazotised and coupled to the second naphthalene component.

According to the present invention a process for the production of a cyan dyestuff image in a photographic layer comprises including in a light-sensitive gelatino silver halide emulsion layer, or in a plain gelatin layer coated adjacent thereto, a cyan dyestuff of the general Formula I, forming a latent silver image in said layer, developing said image, subjecting the developed image to treatment which bleaches or removes the silver image and simultaneously bleaches the dyestuff in situ therewith, and removing any residual silver and silver salts from the product.

The invention further includes photographic materials which comprise a sheet support and a photographic silver halide emulsion layer, the said layer, or a layer adjacent thereto, including a cyan dyestuff of general Formula I.

Further the invention includes photographic materials which comprise, in superposition on a sheet support, a layer of a photographic silver halide emulsion layer sensitive to blue light, a layer of a photographic silver halide emulsion layer sensitised to green light and a layer of a photographic silver halide emulsion layer sensitive to red light, the said layers selectively containing yellow, magenta and cyan dyes, the cyan dye being a dye of general Formula I.

The following are illustrative of the production of dye-stuffs of the present invention:

## EXAMPLE 1



18.2 parts of 6-nitro-3-amino-4-methoxy-1-methyl benzene is slurried with 35 parts of water at 50° C. 32.5 parts of 32% hydrochloric acid is added and after diluting the thick mixture with 10 parts of water the mixture is stirred at 50° C. for 1 hour. The mixture is cooled to 10° C. by external cooling, and then 25 parts of ice is added. Diazotisation is effected by adding a solution of 6.9 parts of sodium nitrite dissolved in 50 parts of water, dropwise, as rapidly as absorbed at a temperature not exceeding 10° C. Diazotisation is essentially complete when an excess of nitrous acid is still detectable by means of starch/iodide test paper, fifteen minutes after the last addition of sodium nitrite. The excess nitrous acid is destroyed by adding a sufficient amount of sulphamic acid. The diazotisation solution is filtered to remove a trace of insoluble matter.

32.0 parts of 1:8-dihydroxynaphthalene-3:6-disulphonic acid is dissolved in 200 parts of water at room temperature and the solution neutralised to Brilliant Yellow test paper by adding 14.2 parts of 31% sodium hydroxide liquor. 20 parts of sodium acetate crystals is added and the solution cooled externally to 5° C.

The diazotisation solution is added dropwise to the stirred solution of 1:8-dihydroxynaphthalene-3:6-disulphonic acid at 5-10° C. during 20 minutes, and the mixture then allowed to stir for a further 15 hours at room temperature. 50 parts of common salt is added, and after stirring for 1 hour the mixture is filtered and the filter paste is washed on the filter with 100 parts of 10% brine.

There results 190 parts of paste nitromonoazo compound which is slurried out in 1200 parts of water and neutralised to litmus with 6.6 parts of 31% sodium hydroxide liquor. The solution is heated to 40-45° C. and a solution of 46 parts of sodium sulphite crystals (Na2S·9H2O) in 40 parts of water is added dropwise with stirring during 1½ hours at 40-45° C. The mixture is stirred for a further 2 hours at 40-45° C. and then screened to remove some insoluble matter. The liquor is cooled to 30° C. and 25 parts of sodium bicarbonate added to precipitate the aminomonoazo compound which is filtered off. There results 87.3 parts of paste aminomonoazo compound equivalent to 37.2 parts of 100% aminomonoazo compound.

12.1 parts of aminoazo compound at 100% is dissolved in 140 parts of water and 6.6 parts of 31% sodium hydroxide liquor and the solution is cooled to below 5° C. by external cooling and 11.6 parts of 32% hydrochloric acid is added to precipitate the aminomonoazo compound in a suitable physical form for diazotisation. Diazotisation is effected by adding dropwise a solution of 1.75 parts of sodium nitrite dissolved in 12 parts of water as fast as absorbed at below 5° C. Diazotisation is considered complete when an excess of nitrous acid is detectable half an hour after the last addition of sodium nitrite.

11.45 parts of 1-amino-8-naphthol-3:6-disulphondiethylamide (equivalent to 10.8 parts of 100%) is dissolved in 140 parts of water with the addition of 6.65 parts of 31% sodium hydroxide liquor. 5 parts of sodium carbonate is added and the solution is cooled externally to 0° C.

35 parts of common salt is added to the slurry of diazotised aminomonoazo compound and the mixture added dropwise to the stirred solution of 1-amino-8-naphthol-3:6-disulphondiethylamide at 0-2° C. over ¾ hour. The

mixture is stirred for 15 hours at below 5° C. and the precipitated disazo dye is filtered off. The paste dye is stirred with 600 parts of water at 60° C. and 60 parts of common salt added to precipitate the dye. The dye is filtered off and washed on the filter with 25% potassium acetate liquor until the dye is free from chloride. The dye is finally washed with 200 parts of isopropanol and dried. There results 10.0 parts of dye.

The 1 - amino-8-naphthol-3:6-disulphondiethylamide may be prepared by the method described in specification No. 615,606.

## EXAMPLE 2



15 The aminomonoazo compound, prepared as described in Example 1, 6.05 parts at 100% is dissolved in 70 parts of water by the addition of 3.3 parts of 31% sodium hydroxide liquor and the solution cooled to below 5° C. by external cooling. 5.85 parts of 32% hydrochloric acid is added and diazotisation effected by the dropwise addition of a solution of 0.875 parts of sodium nitrite dissolved in 6 parts of water as fast as absorbed at below 5° C. Diazotisation is considered complete when an excess of nitrous acid is detectable ½ hour after the last addition of sodium nitrite.

40 4.32 parts of 1-amino-8-naphthol-3:6-disulphonmethylamide at 100% is dissolved in 20 parts of pyridine and 4.45 parts of ammonia liquor, sp. gr. 0.890, and the solution cooled to below 5° C. The slurry of diazotised aminomonoazo compound is added dropwise to the stirred solution over ½ hour at below 5° C. After stirring a further 2 hours at below 5° C., the precipitated dye is filtered off. The paste dye is heated with 500 parts of 20% aqueous isopropanol to 70° C. and then allowed to cool and crystallise. 5 parts of potassium acetate is added and the precipitated dye filtered off. The dye paste is washed on the filter with acetone and the dye dried. There results 4.2 parts of dye.

The 1 - amino - 8-naphthol-3:6-disulphonmethylamide may be prepared in an analogous manner to the method of specification No. 615,606.

## EXAMPLE 3



55 This dye is prepared as described in Example 2 except that 4.7 parts of 1-amino-8-naphthol-3:6-disulphonethylamide is used in the place of 1-amino-8-naphthol-3:6-disulphonmethylamide. There results 3.9 parts of dye.

60 The 1-amino-8-naphthol-3:6-disulphonethylamide may be prepared in an analogous manner to the method of specification No. 615,606.

## EXAMPLE 4



65 This dye is prepared as described in Example 2 except that 4.7 parts of 1-amino-8-naphthol-3:6-disulphonmethylamide is used in place of the 1-amino-8-naphthol-3:6-disulphonmethylamide. There results 3.7 parts of dye.

The 1-amino-8-naphthol-3:6 - disulphondimethylamide may be prepared in an analogous manner to the method of specification No. 615,606.

## EXAMPLE 5



The dye is prepared in a similar way to that described in Example 2 except that 4.67 parts of 1-amino-8-naphthol-4:6-disulphonethylamide is used in place of 1-amino-8-naphthol-3:6 - disulphonmethylamide. There results 10.1 parts of dye.

The 1-amino-8-naphthol-4:6-disulphonethylamide may be prepared in an analogous manner to the methods of specifications Nos. 326,226 and 615,606.

## EXAMPLE 6



The dye is prepared in a similar way to that described in Example 2 except that 5.36 parts of 1-amino-8-naphthol-4:6 - disulphondiethylamide is used in place of 1-amino-8-naphthol-3:6-disulphonmethylamide. There results 10.7 parts of dye.

The 1-amino-8-naphthol-4:6 - disulphondiethylamide may be prepared in an analogous manner to the methods of specifications Nos. 326,226 and 615,606.

## EXAMPLE 7



4.95 parts of 4-nitro-2:5-dimethoxy-1-amino benzene is slurried with a mixture of 8.12 parts 32% hydrochloric acid and 11.0 parts water and cooled to 5° C. by external cooling. Diazotisation is effected by adding a solution of 1.73 parts of sodium nitrite dissolved in 12 parts of water, dropwise, as rapidly as absorbed at a temperature not exceeding 10° C. Diazotisation is essentially complete when an excess of nitrous acid is still detectable by means of starch/iodide test paper, fifteen minutes after the last addition of sodium nitrite. The excess nitrous acid is destroyed by adding just sufficient an amount of sulphamic acid. The reddish brown solution is filtered to remove traces of insoluble matter.

8.5 parts of 1:8-dihydroxynaphthalene-3:6-disulphonic acid is dissolved in 50 parts of water at room temperature and the solution made weakly alkaline to Brilliant Yellow test paper by adding 4.0 parts of 31% sodium hydroxide liquor. 8.0 parts of sodium acetate crystals is added and the solution cooled to below 10° C. by external cooling.

The diazotisation solution is added dropwise to the stirred solution of 1:8-dihydroxynaphthalene-3:6-disulphonic acid at 5-10° C. during 20 minutes and the mixture then allowed to stir for a further 15 hours at room temperature. 10 parts of common salt is added and after stirring for 1 hour the mixture is filtered.

There results 55 parts of paste nitromonoazo compound which is dissolved in 500 parts of water by adding 2.7 parts of 31% sodium hydroxide liquor to make weak-

ly alkaline to litmus test paper. The solution is warmed to 40-45° C. and a solution of 27 parts of sodium sulphide crystals (Na2S·9H2O) in 27 parts of water is added dropwise with stirring during 2 hours at 40-45° C. The reaction mixture is stirred at 40-45° C. for a further 2 hours and then filtered to remove traces of insoluble matter. The solution is cooled to 30° C. and 10.0 parts sodium bicarbonate is added to precipitate the aminomonoazo compound which is filtered off. There results 23.0 parts of paste aminomonoazo compound.

10 16.5 parts of the paste aminomonoazo compound is dissolved in 190 parts of water by adding 3.6 parts of 31% sodium hydroxide liquor and the solution filtered to remove a trace of insoluble matter. The solution is cooled to below 5° C. by external cooling and 7.0 parts of 32% hydrochloric acid is added. A solution of 0.76 part of sodium nitrite dissolved in 5.0 parts of water is added dropwise at 5° C. or below over 20 minutes. The mixture is stirred at below 5° C. for a further 2 hours.

15 20 10.8 parts of 1-amino-8-naphthol-3:6-disulphondiethylamide is dissolved in 100 parts of water, 25 parts of 74° OP industrial methylated spirits and 4.0 parts of 31% sodium hydroxide liquor. 5.0 parts of sodium carbonate is added and the precipitate which forms is redissolved 25 by adding a further 2.0 parts of 31% sodium hydroxide liquor. The solution is cooled to below 5° C.

25 The slurry of diazotised aminomonoazo compound is added dropwise to the stirred solution of 1-amino-8-naphthol-3:6-disulphondiethylamide at 0-5° C. over 1 hour. 30 After stirring for a further one hour the mixture is heated to 90° C. and stirred at 90° C. for 1 hour. The mixture is cooled to 60° C. and 9.5 parts 31% sodium hydroxide liquor is added. The mixture is filtered and washed on the filter with 5% brine made alkaline to Clayton Yellow 35 test paper with sodium hydroxide. The paste dye is slurried with 5% potassium acetate solution, neutralised by adding acetic acid and refiltered. The paste dye is finally washed on the filter with 74° OP industrial methylated spirits and dried at 80° C. in an oven. There results 8.1 parts of dye.

## EXAMPLE 8



45 50 5.76 parts of 4-acetylamo-5-methoxy-2-methyl-1-amino-benzene hydrochloride is dissolved in a mixture of 75 parts of water and 5.8 parts of 32% hydrochloric acid at below 5° C. A solution of 1.73 parts of sodium nitrite dissolved in 12 parts of water is added dropwise as rapidly as absorbed at below 5° C. Diazotisation is essentially complete when an excess of nitrous acid is still detectable by means of starch/iodide test paper, fifteen minutes after the last addition of sodium nitrite. The excess nitrous acid is destroyed by adding just sufficient an amount of sulphamic acid.

55 60 65 8.0 parts of 1:8-dihydroxynaphthalene-3:6-disulphonic acid is dissolved in 100 parts of water by adding 6.7 parts of 31% sodium hydroxide liquor. 10 parts of sodium acetate crystals is added and the solution cooled to below 5° C. The diazotisation liquor is added dropwise to the stirred solution of 1:8-dihydroxynaphthalene-3:6-disulphonic acid over 1/2 hour and the mixture stirred for a further 4 hours. 34 parts of common salt is added and the mixture filtered and the paste acetylaminomonoazo compound washed on the filter with 20% brine.

70 75 The resulting 33.7 parts of paste acetylaminomonoazo compound is dissolved in 125 parts of water and made just alkaline to Brilliant Yellow test paper with the addition of 6.7 parts of 31% sodium hydroxide liquor. A fur-

ther 6.7 parts of 31% sodium hydroxide liquor is added and the solution is heated to 90° C. The mixture is stirred at 90° C. for 5 hours, cooled to 30° C. and 8.5 parts of sodium bicarbonate is added. The precipitated aminomonoazo compound is filtered off.

The paste aminomonoazo compound is dissolved in 125 parts of water by adding 6.7 parts of 31% sodium hydroxide liquor and cooled to below 5° C. 14.5 parts of 32% hydrochloric acid is added and diazotisation is effected by the dropwise addition of a solution of 1.11 parts of sodium nitrite dissolved in 7 parts of water at below 5° C.

11.4 parts of 1-amino-8-naphthol-3:6-disulphondiethylamide is dissolved in a mixture of 40 parts of pyridine and 11.2 parts of ammonia liquor S.G. 0.890 and the solution cooled to below 5° C.

The slurry of the diazomonoazo compound is added dropwise to the stirred solution of 1-amino-8-naphthol-3:6-disulphondiethylamide over 15 minutes at below 5° C. The mixture is stirred for a further 15 hours, heated to 80° C. and 2 parts of sodium carbonate is added. The precipitated dye is filtered off and crystallised from 500 parts of 2½% brine. The crystallised dye is washed with 25% potassium acetate solution and then washed with methylated spirit. The dye is dried at 40° C. There results 11.1 parts of dye.

Further, according to the invention, a process of colour photography comprises a process as set forth above in which the gelatino silver halide layer is red-sensitive and constitutes one of the layers of a multilayer photographic material which further contains photographic emulsion layers sensitive to green and blue light and respectively dyes with magenta and yellow dyestuffs, and the said cyan dyestuff is included in said red-sensitive layer or in a plain gelatin layer coated adjacent thereto. More particularly the invention provides a process in which the said cyan dyed layer is layer (b) of an assembly consisting of:

- (a) Support layer
- (b) Red-sensitive emulsion layer dyed cyan
- (c) Green-sensitive emulsion layer dyed magenta
- (d) Blue-absorbing filter layer
- (e) Blue-sensitive emulsion layer dyed yellow, optionally with plain colloid separating layers between some or all of the adjacent layers recited.

The invention further includes such light-sensitive materials employed in the aforesaid processes, and suitable for variants of those processes, which consist of or include a gelatino silver halide emulsion layer containing a cyan dyestuff as above set forth.

The bleaching of the cyan dyestuffs employed in this invention can be effected by any of the types of bleaching bath commonly employed in the silver-dye-bleach process.

The plain use of acid, e.g. hydrobromic or hydrochloric, is effective but is very slow. The inclusion of halide salts has an accelerative effect, but these bleaching baths are still slow. The inclusion of a solvent for silver halide such as thiourea or pyridine has a strongly accelerative effect, and this can be greatly increased by the inclusion of an accelerating substance or catalyst. In these connections reference may be made to British patent specifications Nos. 397,159 and 490,451 for suitable bleaching baths.

The following example, which for simplicity is concerned only with the treatment of a single layer containing the cyan dyestuff, will serve to illustrate this aspect of the invention:

#### EXAMPLE 9

1.80 gms. of the cyan dyestuff of Example 1 are dissolved in 180 mls. of distilled water. This solution is added to 820 mls. of silver chlorobromide emulsion containing 1.62 gms. silver as silver halide. The mixture is coated on film to give a coating weight of 1.3 mgms. of silver (as silver halide) per square decimetre.

The dried coating is exposed to light to record an image therein and processed at 68° F. as follows:

(1) Develop to a silver image by two minutes' treatment in the following developer:

|                           | Gms. |
|---------------------------|------|
| Metol                     | 0.75 |
| Sodium sulphite (cryst.)  | 25   |
| Hydroquinone              | 3    |
| Sodium carbonate (cryst.) | 40   |
| Potassium bromide         | 1    |
| Water to 1 litre.         |      |

- (2) Rinse 30 seconds.
- (3) Fix in 20% sodium thiosulphate for 3 minutes.
- (4) Rinse 30 seconds.
- (5) Harden in 4% formalin.
- (6) Wash 10 minutes.
- (7) Dye-bleach for 8 minutes in the following bath:

|                               |     |      |
|-------------------------------|-----|------|
| Hydrochloric acid (S.G. 1.19) | ccs | 100  |
| Potassium bromide             | gms | 12.5 |
| Thiourea                      | gms | 10   |
| 2:3-dimethyl quinoxaline      | gms | 0.1  |
| Water to 1 litre.             |     |      |

- (8) Wash 5 minutes.
  - (9) Silver-bleach for 5 minutes in the following bath:
- |                           |     |     |
|---------------------------|-----|-----|
| Copper sulphate (cryst.)  | gms | 100 |
| Sodium chloride           | gms | 100 |
| Hydrochloric acid (conc.) | ccs | 50  |
| Water to 1 litre.         |     |     |
- (10) Wash 5 minutes.
  - (11) Fix in 20% sodium thiosulphate for 3 minutes.
  - (12) Wash for 10 minutes and dry.

A reverse image in cyan dye is obtained.

Steps 4 and 5 may be omitted if the original emulsion is hardened or provided with a hardened gelatin supercoat.

Similar results are obtained using the other dyestuffs falling within the general Formula I.

When the process is repeated with a gelatin coating containing dye but not silver halide, it is found that substantially the same density of dye can be measured after processing as before.

All the said dyestuffs have good resistance to migration, bleach rapidly and effectively and are much superior in colorimetric characteristics to cyan dyestuffs hitherto employed for the purpose.

The following table shows examples of further dyes suitable for incorporation in a red sensitive photographic layer as exemplified by Example 9. The table lists the components of the dyes as first, middle and end components and the dyes are prepared by a method essentially the same as that described in Example 1.

|    | 1st component                                  | Middle component                            | End component                                 |
|----|------------------------------------------------|---------------------------------------------|-----------------------------------------------|
| 1. | 1:8-dihydroxynaphthalene-3:6-disulphonic acid. | 6-nitro-3-amino-4-octyloxy-1-methylbenzene. | 1-amino-8-naphthol-3:6-disulphondiethylamide. |
| 2. | 1:8-dihydroxynaphthalene-3:6-disulphonic acid. | 6-nitro-3-amino-4-chloro-1-methoxybenzene.  | Do.                                           |
| 3. | 1:8-dihydroxynaphthalene-3:6-disulphonic acid. | 4-nitro-1-amino benzene-2-sulphonic acid.   | Do.                                           |
| 4. | 1:8-dihydroxynaphthalene-3:6-disulphonic acid. | 6-nitro-3-amino-1:4-dichlorobenzene.        | Do.                                           |
| 5. | 1:8-dihydroxynaphthalene-3:6-disulphonic acid. | 6-nitro-3-amino-4-methoxy-1-methylbenzene.  | Do.                                           |
| 6. | 1:8-dihydroxynaphthalene-3:6-disulphonic acid. | do.                                         | Do.                                           |
| 7. | 1:8-dihydroxynaphthalene-3:6-disulphonic acid. | do.                                         | 1-naphthol-4-sulphondiethylamide.             |

I claim as my invention:

1. A process for the production of a cyan dyestuff image in a photographic silver halide emulsion layer

which comprises including in contact with said emulsion a cyan dyestuff selected from the class consisting of dye-stuffs of the formula:



where X is selected from the class consisting of halogen, hydroxyl, amino, substituted amino and hydrogen, U is selected from the class consisting of hydrogen, sulphonic acid and alkali metal sulphonate, V is selected from the class consisting of hydrogen and the grouping:



and  $R_1$  and  $R_2$  taken separately are each selected from the class consisting of hydrogen, alkyl, substituted alkyl, cycloalkyl, aralkyl and aryl and taken together constitute, with the nitrogen atom to which they are attached, a cyclic grouping, and the said dyestuffs in which the ring  $W$  carries at least one substituent selected from the class consisting of halogen, alkyl, alkoxy, sulphonate acid and alkali metal sulphonate, the number of sulphonate groups in the ring  $W$  being not greater than 1, forming a latent silver image in said emulsion layer, developing said image, subjecting the developed image to treatment which bleaches the silver image and simultaneously bleaches the said dyestuff in situ therewith, and removing any residual silver and silver salts from the product.

2. A photographic material which comprises a sheet support and a photographic silver halide emulsion layer, including in contact with said emulsion a cyan dyestuff selected from the class consisting of dyestuffs of the formula:



where X is selected from the class consisting of halogen, hydroxyl, amino, substituted amino and hydrogen, U is selected from the class consisting of hydrogen, sulphonic acid and alkali metal sulphonate, V is selected from the class consisting of hydrogen and the grouping:



and  $R_1$  and  $R_2$  taken separately are each selected from the class consisting of hydrogen, alkyl, substituted alkyl, cycloalkyl, aralkyl and aryl and taken together constitute, with the nitrogen atom to which they are attached, a cyclic grouping, and the said dyestuffs in which the ring  $W$  carries at least one substituent selected from the class consisting of halogen, alkyl, alkoxy, sulphonate acid and alkali metal sulphonate, the number of sulphonate groups in the ring  $W$  being not greater than 1.

3. A photographic material which comprises a sheet support and, in superposition thereon, a layer of a photographic silver halide emulsion sensitive to blue light, a layer of a photographic silver halide emulsion sensitive to green light and a layer of a photographic silver halide emulsion sensitive to red light, the said layers selectively

containing yellow, magenta and cyan dyes and the cyan dye being a dye of the formula:



10 where X is selected from the class consisting of halogen, hydroxyl, amino, substituted amino and hydrogen, U is selected from the class consisting of hydrogen, sulphonic acid and alkali metal sulphonate, V is selected from the  
15 class consisting of hydrogen and the grouping:



20 and  $R_1$  and  $R_2$  taken separately are each selected from the class consisting of hydrogen, alkyl, substituted alkyl, cycloalkyl, aralkyl and aryl and taken together constitute, with the nitrogen atom to which they are attached, a cyclic grouping and the said dyestuffs in which the ring

25 W carries at least one substituent selected from the class consisting of halogen, alkyl, alkoxy, sulphonic acid and alkali metal sulphonate, the number of sulphonic groups in the ring W being not greater than 1.

4. A photographic material according to claim 3  
30 wherein the cyan dye is a dye of the formula:



5. A photographic material according to claim 3  
40 wherein the cyan dye is a dye of the formula:



6. A photographic material according to claim 3 wherein the cyan dye is a dye of the formula:



7. A photographic material according to claim 3 wherein the cyan dye is a dye of the formula:



8. A photographic material according to claim 3, wherein the cyan dye is a dye of the formula:



11

9. A photographic material according to claim 3 wherein the cyan dye is a dye of the formula:



10. A photographic material according to claim 3 wherein the cyan dye is a dye of the formula:



12

11. A photographic material according to claim 3 wherein the cyan dye is a dye of the formula:



#### References Cited by the Examiner

##### UNITED STATES PATENTS

|           |         |               |         |
|-----------|---------|---------------|---------|
| 1,975,609 | 10/1934 | Knight        | 260—190 |
| 2,612,448 | 9/1952  | Gasper et al. | 96—73   |
| 2,779,758 | 1/1957  | Neier et al.  | 260—290 |
| 3,038,802 | 6/1962  | Keller et al. | 96—73   |
| 3,211,554 | 10/1965 | Dreyfuss      | 96—99   |

##### FOREIGN PATENTS

|         |         |               |  |
|---------|---------|---------------|--|
| 479,607 | 12/1951 | Canada        |  |
| 615,606 | 1/1949  | Great Britain |  |

##### OTHER REFERENCES

Venkataraman: "Synthetic Dyes," vol. II, page 1221, Academic Press, Inc., New York (1952).

NORMAN G. TORCHIN, Primary Examiner.

J. T. BROWN, Assistant Examiner.